# EUROPEAN PATENT SPECIFICATION

(11) **EP 0 677 604 B1**
(45) Date of publication and mention of the grant of the patent: **21.10.1998**
(21) Application number: 94111365.6
(22) Date of filing: 21.07.1994
(51) Int. Cl.: D04B 1/18

(54) **Elastic double-knit fabric**
Elastisches Doppelgestrick
Tricot double élastique

(30) Priority: 12.04.1994 WO PCT/US94/03992
(43) Date of publication of application: 18.10.1995
(73) Proprietor: E.I. DU PONT DE NEMOURS AND COMPANY, Wilmington Delaware 19898 (US)
(72) Inventor: Michel, Gérard Henri Ferdinand, CH-1217 Meyrin/GE (CH)
(74) Representative: von Kreisler, Alek, Dipl.-Chem.

(56) References cited:
- EP-A- 0 498 062
- BE-A- 704 681
- DE-U- 9 305 795
- FR-A- 2 653 789
- US-A- 4 062 204
- MELLIAND TEXTILBERICHTE, vol. 73, no. 10, October 1992 HEIDELBERG, pages 812-815, XP 000310466 KUNDE 'Elastomerverarbeitung auf Rundstrickmaschinen 000310466'

## Description

### Background of Invention

### Field of Invention:

This invention relates to elastic double-knit fabrics and more particularly to elastic double-faced weft-knit fabrics.

### Background:

It is well-known to knit elastic yarns such as spandex yarns with hard yarns to produce knitted fabrics having a certain amount of "ive". Heretofore, elastic double-knit fabrics have been made in one of two ways. One, the elastic yarn is plaited with a hard yarn on the same feed on both the dial and cylinder. Such a fabric is heavy, costly, and requires heat stabilization to obtain a fabric which can be used commercially. Second, the fabric weight and cost can be lowered by plaiting the elastic yarn with a hard yarn either on the dial or cylinder only. However, such a fabric still must be heat-set.

US Patent No. 4,062,204 discloses a fabric comprising rigid synthetic yarns with no previous texturing or warping, which as producer twists or rigid yarns are pique knitted on the basis of interchanging courses of interlock and jersey; and annexed to the rigid yarn forming the courses of jersey stitches there is an elastomeric fiber of polyurethane origin under controlled tension.

Further background art is Melliand Textilberichte, vol. 73, no. 10, October 1992 Heidelberg, pages 812-815, XP 000310466 Kunde "Elastomerverarbeitung auf Rundstrickmaschinen"; FR-A-2 653 789; BE-A-704 681; EP-A-0 498 062; DE-U-93 05 795.

It has now been found that, if the elastic yarn is plaited independently on the dial of the first feed and the cylinder of the second feed with independent hard yarns, the above-mentioned difficulties are overcome. In addition, such anew fabric has hither power at a lower elongation. For double-faced double-knit fabrics, a light-weight fabric is now possible; and it does not have to be heat-set prior to use.

### Summary of the Invention

According to the present invention there is provided a double-knit fabric made from elastic yarns and hard yarns characterized in that two independent elastic yarns are plaited with independent hard yarns or filaments, one elastic yarn plaited with a hard yarn or filament on the dial of a first feed and the second elastic yarn plaited with a second hard yarn or filament on the cylinder of a second feed.

### Brief Description of the Drawings

The drawing diagrammatically illustrates the first six courses of a double knit plain rib fabric produced on a circular knitting machine.

### Detailed Description of the Invention

In accordance with the invention, elastic yarns and hard yarns are knitted so as to provide a double-knit fabric which does not have to be heat-set after knitting. Thus, the final knitted fabric weight and width is obtained on the machine.

The terms "elastic" yarn and "hard" yarn or filament as used herein are well-known in the art. Examples of suitable "elastic" yarns including shirring elastic and various elastane fibers, particularly those sold under the tradename LYCRA. A "hard" yarn is a non-contractible yarn and there is a wide range of such yarns that can be used in this invention, both natural and synthetic. The "hard" yarn(s) or filament(s) used will be selected primarily for the visual appearance and feel of the final fabric. Suitable natural spun yarns are cotton, linen, wool, cashmere, alpaca, silk, mohair, and blends of any of them. Suitable synthetic spun yarns include polyester, polyamide, and viscose. The synthetic yarns can also be blended with natural yarns such as cotton/polyester or wool/polyester. A filament is typically a continuous filament yarn of a synthetic polymer such as a polyester or a polyamide.

The double-knit fabric of the present invention can be knitted on any of the conventional circular knitting machines used for double-knits. These machines and constructions are well-known to those skilled in the art.

As shown in the drawing, in the first, third, and fifth courses, an elastic yarn 1 is fed independently to the cylinder only of a circular knitting machine. The yarn is fed under tension with a hard yarn 2 and plaited with it. In the second fourth and sixth courses, a second elastic yarn 3 is fed under tension to the dial only of a circular knitting machine and is plaited with hard yarn 4. Courses 1 and 2 are repeated for as long as desired to make a plain rib fabric. As stated earlier, the appearance and feel of the fabric can be varied by selecting different hard yarns and by varying the dtex of the yarns used. In addition, different fabric constructions can be prepared by varying the needle selection. Constructions according to the invention will be called the "Meyrinoise Stitch".

The invention can be further illustrated by the following examples:

### Example 1

A 1/1 plain rib double-knit fabric as shown in the drawing was made on a TERROT 20-gauge circular knitting machine having a 30 inch (76.2 cm) diameter and 2 X 1872 needles. The elastic yarns independently fed to the dial and cylinder of the knitting machine were 78 dtex LYCRA (elastane) and the hard yarns independently fed with the elastane yarns were 85/1 number metric (Nm) cotton. The resulting plain rib fabric contained 12% by weight elastane and 88% by weight cotton, had a finished weight of 158 g/m2, and had a finished width of 170 cm. This fabric was ready for standard dyeing and finishing conditions used for hard yarns without heat-setting.

### Example 2

Using the same circular knitting machine as in Example 1, except set for an interlock construction, two 22 dtex elastane yarns and the same cotton yarns were fed independently as shown in the drawing. The resulting interlock fabric contained 4% by weight elastane and 96% by weight cotton, had a finished weight of 244 g/m2, and had a finished width of 96 cm. This fabric was ready for standard dyeing and finishing conditions used for hard yarns without heat-setting.

## Claims

1. A double-knit fabric made from elastic yarns (1,3) and hard yarns (2,4) characterized in that two independent elastic yarns (1,3) are plaited with independent hard yarns or filaments (2,4), one elastic yarn (3) plaited with a hard yarn or filament (4) on the dial of a first feed and the second elastic yarn (1) plaited with a second hard yarn or filament (2) on the cylinder of a second feed.

2. A double-knit fabric according to Claim 1 wherein the elastic yarns (1,3) are elastane yarns.

3. A double-knit fabric according to Claim 1 or Claim 2 wherein the hard yarns or filaments (2,4) are yarns and are the same.

4. A double knit fabric according to Claim 1 or Claim 2 wherein the hard yarn or filament (4) of the first feed is different from the hard yarn or filament (2) of the second feed.

5. A double-knit fabric according to Claim 4 wherein one of the hard yarns or filaments (2,4) is a continuous filament so as to provide a double-faced double-knit fabric.

6. A double-knit fabric according to any of Claims 1 to 5 wherein the fabric has a plain rib-based construction.

7. A double-knit fabric according to any of Claims 1 to 5 wherein the fabric has an interlock-based construction.

## Patentansprüche

1. Doppeltrikot, das aus elastischen Garnen (1, 3) und harten Garnen (2, 4) hergestellt ist, dadurch gekennzeichnet, daß zwei unabhängige elastische Garne (1, 3) mit unabhängigen harten Garnen oder Filamenten (2, 4) verflochten sind, wobei das eine elastische Garn (3) auf der Rippscheibe einer ersten Zuführung mit einem harten Garn oder Filament (4) verflochten wird und das zweite elastische Garn (1) auf dem Zylinder einer zweiten Zuführung mit einem zweiten harten Garn oder Filament (2) verflochten wird.

2. Doppeltrikot gemäß Anspruch 1, wobei die elastischen Garne (1, 3) Elastangarne sind.

3. Doppeltrikot gemäß Anspruch 1 oder 2, wobei die harten Garne oder Filamente (2, 4) Garne sind und gleich sind.

4. Doppeltrikot gemäß Anspruch 1 oder 2, wobei das harte Garn oder Filament (4) der ersten Zuführung von dem harten Garn oder Filament (2) der zweiten Zuführung verschieden ist.

5. Doppeltrikot gemäß Anspruch 4, wobei eines der harten Garne oder Filamente (2, 4) ein endloses Filament ist, so daß man ein doppelseitiges Doppeltrikot erhält.

6. Doppeltrikot gemäß einem der Ansprüche 1 bis 5, wobei der Stoff einen auf Einfachrippen basierenden Aufbau hat.

7. Doppeltrikot gemäß einem der Ansprüche 1 bis 5, wobei der Stoff einen auf Doppelrippen (Interlock) basierenden Aufbau hat.

## Revendications

1. Tricot double constitué de fils élastiques (1,3) et de fils rigides (2,4), caractérisé en ce que deux fils élastiques indépendants (1,3) sont vanisés avec des fils ou filaments rigides indépendants (2,4), un fil élastique (3) étant vanisé avec un fil ou filament rigide (4) sur le disque à côtes d'une première alimentation et le second fil élastique (1) étant vanisé avec un second fil ou filament rigide (2) sur le cylindre d'une seconde alimentation.

2. Tricot double selon la revendication 1, dans lequel les fils élastiques (1,3) sont des fils d'élasthanne.

3. Tricot double selon la revendication 1 ou 2, dans lequel les fils ou filaments rigides (2,4) sont des fils et sont identiques.

4. Tricot double selon la revendication 1 ou 2, dans lequel le fil ou filament rigide (4) de la première alimentation est différent du fil ou filament rigide (2) de la seconde alimentation.

5. Tricot double selon la revendication 4, dans lequel l'un des fils ou filaments rigides (2,4) est un filament continu de manière à obtenir un tricot double double face.

6. Tricot double selon l'une quelconque des revendications 1 à 5, dans lequel le tissu a une structure à base de côtes fines.

7. Tricot double selon l'une quelconque des revendications 1 à 5, dans lequel le tissu a une structure à base d'interlock.
